

Jan. 18, 1927.

1,614,506

C. C. VAN VOORHIS

ELECTRICAL DEVICE

Filed Feb. 16, 1922



INVENTOR  
CLETUS C. VAN VOORHIS

BY  
*J. F. Gilbert*  
ATTORNEY

Patented Jan. 18, 1927.

## UNITED STATES PATENT OFFICE.

CLETUS CLINTON VAN VOORHIS, OF EAST ORANGE, NEW JERSEY, ASSIGNEE TO  
WESTINGHOUSE LAMP COMPANY, A CORPORATION OF PENNSYLVANIA.

## ELECTRICAL DEVICE.

Application filed February 16, 1922. Serial No. 536,942.

This invention relates to electrical lamps and more particularly to lamps filled with a rare gas and which are termed discharge, gas or glow lamps.

5 Gas lamps, especially those having a filling of neon gas, find considerable use for ornamental purposes or for sign lighting, and are particularly advantageous when used as small indicating or pilot lamps.

10 These lamps employ a relatively low current and, when they are operated on commercial circuits, it is desirable to provide a resistance in series with each lamp for the purpose of preventing the passage of excessive currents

15 therethrough. The stabilizing resistances frequently employed consist of separate units disposed in the line or of a separate resistance element of such character as to be contained either in the interior of the lamp

20 or in the base thereof. My invention concerns itself with improving this part of the lamp.

One of the objects of my invention is to provide a lamp with a stabilizing resistance element which may constitute an integral part of a lamp.

Another object of my invention is the provision of an element which will serve a double purpose, namely, that of a stabilizing 30 resistance and as an adhesive medium for securing one portion of a lamp to another.

A further object is the provision of a basing cement which will also serve as a resisting medium.

35 The above objects may be accomplished by providing a resistance material having an adhesive property necessary to a cement and capable of serving to unite the base of the lamp to the bulb. It is common, in the art 40 of manufacturing electric lamps, to secure the base or screw cap to the bulb or envelope in which the source of light is disposed by an interposed layer of cement. This cement, which is termed a basing cement, is 45 usually of a suitable consistency to permit its flow into the base. In practice, the base and bulb are properly juxtaposed until the cement is pressed against the surface of the bulb and the inner surface of the base, after 50 which the cement is hardened by baking, thus bonding the base and the bulb.

In practicing my invention, I employ a suitable basing cement and combine therewith a conductive material in sufficient proportions to provide a given resistance, the

necessary adhesive property and the plasticity of the cement, previous to baking, being maintained.

By the provision of a resistance element incorporated in the cement, considerable advantage is derived, inasmuch as the necessity for external resistance devices is avoided and no appreciable amount of space is required for my resistance element when incorporated in a lamp.

55 The accompanying drawing illustrates an embodiment of my invention as applied to a lamp, part of the structure being shown in section.

The lamp (partly illustrated) may be of any desired type having an envelope 2 containing a filling of a suitable gas and provided with leading-in wires 3 and 4 which extend from, and are sealed in, a pressed portion 6 of the envelope. The leading-in 70 wires conduct current to electrodes (not shown) disposed within the envelope. The electrodes may be of any suitable form, depending upon the use to be made of the lamp. A hollow threaded member or base 7 is provided and, in lamps of the ordinary 75 type, this base is secured to the envelope by an adhesive medium or basing cement, and one of the leading-in wires of the lamp is connected to the base, the other leading-in 80 wire being connected to an external contact member 8 which is insulated from the shell or body of the base by a separator 9 made of glass or other insulating material.

85 A lamp constructed according to my invention may be provided with a cement constituting a combined resistance and adhesive substance 10 which may be termed a resistance element. An end 11 of the leading-in 90 wire 4 projects from the envelope 2 a sufficient distance to permit a portion and, consequently a given area of the wire, to make contact with the resistance element 10. The leading-in wire 3 extends through the resistance element and the base 7 and is soldered, or otherwise secured, to the contact 95 member 8.

100 As illustrated in the accompanying drawing, a portion of the leading-in wire 3 extends through the resistance element or cement 10, which construction necessitates the provision of a layer of insulating material 12 to prevent short circuiting of the current. Such insulation may be of any desired material and may be applied by the most con- 105

venient method. It has, however, been found desirable to employ any suitable insulating varnish or a viscous water solution of sodium silicate which may be applied to the 5 leading-in wire by means of a brush.

When this coating is dry, the layer 12, thus formed, furnishes an efficient insulation. In order to more positively prevent any current from passing through the base 10 adjacent to the end of the leading-in wire 3, a layer 14 of any suitable material as, for instance, glass-wool, asbestos-fiber or the like may be disposed between the end of the base 7 and the resistance element 10. Thus, the 15 contact 8 is more perfectly insulated from the resistance element.

When the invention, as above set forth, is applied to a lamp of well known form, in which a so-called flare seal is employed, 20 there will be, instead of the press 6, as illustrated, a space between the resistance element 10 and the envelope which may be filled with glass-wool or insulating material. This will prevent the resistance element, 25 when in a plastic state, from flowing in contact with leading-in wires.

In practice, the required portion of the leading-in wire 3 is given a coating of the insulating material 12. A predetermined 30 amount of plastic cement, containing the proper proportion of conductive material, is then deposited in a base which is slipped over the end of an envelope or bulb, the leading-in wire 3 being, at the same time, 35 threaded through an aperture in the contact element 8 from which it slightly projects. The cement is then hardened by the usual baking process, after which the end of the leading-in wire 3 is soldered to the contact element 8. When the base containing 40 the cement is applied to the bulb, it is obvious that the leading-in wire 4 which projects from the bulb will be disposed within the cement, consequently, when the cement hardens, a firm contact is secured between the 45 wire and the cement or resistance element 10.

It will be appreciated that the resistance of the cement or resistance element 10 will depend upon several factors, i. e., the diameter 50 and length of the portion of the wire which makes contact with the element, the dimension of the base and the conductivity of the cement or resistance element. The latter factor is dependent upon the materials 55 used to make a cement conductive and the relative amount of these conductive materials used.

The composition which I have found to 60 answer all the requirements preferably consists of a mixture of a suitable filler as, for instance, barium sulphate or marble flour, or both, and a soluble gum such as shellac or Bakelite to which is added a suitable conductive substance, such as a metallic powder, as, for instance, a molybdenum or

tungsten powder or powdered carbon; to this mixture may be added a suitable solvent, such as alcohol, in sufficient proportion to produce a plastic composition of the desired viscosity.

In order to ensure a resistance of about 5000 ohms, using a standard candelabra base, having leading-in wires 4 of 25 mil wire,  $\frac{1}{4}$  inch of one of the wires being in contact with the cement, a cement of the 75 following composition may be used:

|                                                         | Parts by weight. |
|---------------------------------------------------------|------------------|
| Barium sulphate-----                                    | 3                |
| Marble flour-----                                       | 8                |
| Powdered graphite (pulverized electrode graphite) ----- | 80               |
|                                                         | 3                |

The ingredients are intimately mixed and are made sufficiently plastic and adhesive by means of approximately 5 parts of a shellac solution. The barium sulphate, marble flour and powdered graphite are preferably fine enough to pass through a 60-mesh screen. The shellac solution may be prepared by dissolving one pound of powdered bleached shellac in one quart of methyl alcohol or ethyl alcohol denatured with methyl alcohol.

Although I have obtained good results by the use of a shellac solution, it will be evident that, if desirable, the shellac may be mixed with the conductive substance and the filler, a suitable volatile solvent being added to this mixture to produce a plastic composition of appropriate viscosity. When a cement of relatively high temperature resistance is required, Bakelite may be substituted for shellac, but, if a cheaper product is desired, Albertol may be employed as the substitute.

The ingredients are intimately mixed until their consistency is such as to enable the composition to be readily poured or shaped into any desirable form, after which it may be baked until the solvent is volatilized and a relatively rigid tenacious product is obtained.

It will thus be evident that I may prepare the composition of any workable consistency which will permit the composition to be poured and disposed in a given relation to one or more of the component parts of a device which may be secured together by the composition. Electrical conductors may be suitably disposed or embedded in the composition while in its plastic state and thus secured therein when the composition has become hardened by baking.

By the use of my invention, it is possible to manufacture glow lamps of very small size including a stabilizing resistance, and considerable advantage is thereby obtained. When it is desirable to employ a lamp having a small base, it is obvious that the desired results may be had by my compara-

tively simple construction and that a small lamp may be placed in a commercial line without expensive additions in the way of 45

stabilizing resistance devices other than the 5 self contained resistance element within the lamp.

The composition, when prepared in accordance with the above directions, is light 10 in weight, has a high temperature resistance, 10 does not crack in drying and possesses, in a high degree, all the desired properties of a cement and a resistance element.

Since my invention may be embodied in many other forms than that shown and de- 15 scribed, I do not wish to be restricted to the exact form shown but intend to cover all modifications which lie within the scope of the appended claims.

What is claimed is:

20 1. An electric lamp having an envelope, a base, and a resistance element comprising an adhesive substance capable of securing the base to said envelope and serving as a part of a circuit for the passage of electrical 25 energy to said lamp.

2. An electric gas lamp having an envelope and a base, said base being secured to said envelope by a cement capable of serving as a stabilizing resistance.

30 3. An electric gas lamp comprising an envelope, a base for said lamp, a substance for securing said base to said envelope, said substance containing a conductive material whereby the said substance is adapted to 35 serve as a stabilizing resistance.

4. An electric gas lamp comprising an envelope, leading-in wires projecting therefrom, a base for said lamp, a contact element insulated from said base and connected with 40 one of said leading-in wires, a conductive adhesive substance disposed within said base to secure the base to said envelope, an end of the other of said leading-in wires being

embedded in said substance, the other leading-in wire being insulated from said sub- 45 stance.

5. An electric gas lamp comprising an envelope having leading-in wires projecting therefrom, a base secured to said envelope by an adhesive substance containing a conductive material to permit a flow of current 50 from said base to a leading-in wire embedded in said material, a contact member associated with said base, the other leading-in wire being insulated from said material and connected to said contact member, said member being insulated from the body of said base. 55

6. An electric gas lamp comprising a bulb having a base secured thereto by a layer of adhesive resistance material, leading-in wires 60 extending from said bulb, one of said wires being in contact with said material the other wire being insulated from said material.

7. An electric lamp comprising a base, a bulb having one end thereof positioned in 65 said base, leading-in wires extending from said bulb, a layer of adhesive resistance substance interposed between said base and said bulb, an end of one of said leading-in wires connected to an external contact member and 70 the end of the other leading-in wire embedded in said substance.

8. An electric lamp comprising a bulb having a base associated therewith, leading-in wires extending from said bulb, said base 75 being provided with a contact member, one of said leading-in wires being connected to said member, the other leading-in wire projecting a given distance from said bulb, cement within said base and in contact with said last mentioned leading-in wire, said cement having conductive and adherent properties. 80

In testimony whereof, I have hereunto subscribed my name this 15 day of Feb., 1922.

CLETUS CLINTON VAN VOORHIS.